

# United States Patent

[19]

Malizio et al.

[11] 3,905,809

[45] Sept. 16, 1975

[54] ALLOY FOR MAKING DUCTILE IRON

[75] Inventors: Andrew B. Malizio, Delran; Martin A. Rice, Florence, both of N.J.; Harry F. Brooks, Levittown, Pa.

[73] Assignee: United States Pipe and Foundry Company, Birmingham, Ala.

[22] Filed: Jan. 18, 1974

[21] Appl. No.: 434,403

## Related U.S. Application Data

[62] Division of Ser. No. 189,670, Oct. 15, 1971, Pat. No. 3,799,767.

[52] U.S. Cl. .... 75/134 S; 75/53; 75/130 A

[51] Int. Cl. .... C22c 33/00; C21c 7/00; C22c 37/02

[58] Field of Search ..... 75/53, 130 A, 134 S

## [56] References Cited

### UNITED STATES PATENTS

2,814,559 11/1957 Clark ..... 75/53

|           |         |                |          |
|-----------|---------|----------------|----------|
| 2,816,829 | 12/1957 | Bogart .....   | 75/130 A |
| 3,336,118 | 8/1967  | Newitt .....   | 75/58    |
| 3,492,118 | 1/1970  | Mickelson..... | 75/53    |

Primary Examiner—Peter D. Rosenberg  
Attorney, Agent, or Firm—Pennie & Edmonds

[57]

## ABSTRACT

A process for producing ductile iron comprising adding to a bath of low-sulfur cast iron, a material containing at least two graphite-nodularizing elements. The additive material contains each nodularizing element in relatively low concentrations so that after dissolution in the bath the concentration of nodularizing elements remaining is sufficient to produce the desired structure, but the concentration of any one element is, of itself, insufficient to produce nodular (spheroidal) graphite.

4 Claims, 5 Drawing Figures

FIG. 1.  
(PRIOR ART)

FIG. 2.



SHEET 2 OF 3

FIG. 3.



FIG. 4.



F/G. 5.  
(RATE OF FADING OF MAGNESIUM AND CERIUM  
WHEN ADDED TO PIPE IRON IN COMBINATION)



**ALLOY FOR MAKING DUCTILE IRON**

This is a division of application Ser. No. 189,670, filed Oct. 15, 1971, now U.S. Pat. No. 3,799,767.

**BACKGROUND OF THE INVENTION**

The invention is in the field of metallurgy, more specifically, cast iron metallurgy, wherein the end products are ductile iron castings produced by either the permanent mold or sand casting processes.

For many years the major commercial method for the production of ductile iron has been by the addition of magnesium in the form of magnesium-containing alloys or by the addition of the pure element whereby the magnesium causes the graphite to solidify in the form of spheroids. The formation of graphite in this shape is responsible for the outstanding strength and ductility of the material.

There are many well-recognized disadvantages to the use of magnesium or magnesium-containing alloys, chief among them is that the reaction caused by addition of magnesium to molten iron is generally quite violent and accompanied by the formation of thick clouds of white smoke containing magnesium oxide particles. The reaction is also accompanied by brilliant white flare that is harmful to vision. There are further disadvantages in that the high degree of reactivity makes it difficult to obtain a high recovery of the added magnesium, hence the process is inefficient. In addition to the poorer recoveries generally obtainable, the magnesium content of the melt decreases with time due to loss of magnesium from the bath by vaporization, by oxidation and by combination with any sulfur in the bath. The loss of magnesium is generally referred to in the art as "fading."

Certain of the aforementioned disadvantages can be partially overcome depending on the manner of adding the magnesium or Magnesium-alloy to the molten metal bath. For example, flash and flare can be shielded from the eye by a protective cover. Also, somewhat greater efficiencies can be realized when the magnesium is added to the bath under pressure as opposed to pouring the molten metal on top of the magnesium-alloy. These methods are generally undesirable from an economic and process viewpoint in that they require additional equipment to either enclose the area where the magnesium additions are being made or to pressurize the vessel in which the additions are made. Such methods, particularly the pressurizing method, also add additional time and expense to the process.

On the other hand, it is known to the art that cerium is also a nodularizing element and is less reactive upon addition to molten cast iron thus overcoming the flare and smoke problem and also giving increased recoveries. Despite the higher recoveries and lack of reactivity, cerium will still exhibit an undesirably high rate of fade. In addition, cerium is generally only effective in hyper-eutectic cast irons, it is a strong carbide former and, in our experience, has produced graphite particles that are not as perfectly shaped as those produced by the magnesium process.

**SUMMARY OF INVENTION**

The nature of our work has been to develop a process for producing ductile cast iron that would solve some of the problems tolerated by the prior art. One of the objects of our invention is to reduce the amount of

nodularizer required to produce nodular graphite in castings.

Another object of our invention is to reduce the fume and flare accompanying the addition of the nodularizing material.

A further object of our invention is to decrease the rate of "fade" of the nodularizing effect in the treated bath.

Yet another object of our invention is to provide a process for minimizing the dross content of ductile iron.

Also an object of our invention is to provide a process allowing a selection of a number of individual nodularizers and quantities of individual nodularizers.

These objects are achieved in our preferred embodiment by adding to a bath of low sulfur cast iron two or more nodularizers in a silicon-iron alloy or mixture of silicon-iron alloys wherein the alloy or mixture of silicon-alloys contains not more than three per cent of any one nodularizer and the combination of all nodularizers in the alloy or mixture of alloys is not more than 6 per cent with the resultant advantage being:

- a. a drastic reduction in fume and flare when the alloy is added to the bath.
- b. a greatly decreased rate of fade of the nodularizing effect.
- c. a reduction in total nodularizer required for a given casting.
- d. a reduction in the dross content in the castings.

**DESCRIPTION OF DRAWINGS**

FIG. 1 is a schematic representation of the basic steps in the usual process of making ductile iron castings, and is not part of our invention.

FIG. 2 is a graphical representation showing the amount of effective nodularizing elements remaining in a bath of molten iron vs. holding time and comparing additions of one nodularizing element (as known in the prior art) to additions of more than one nodularizing element in accordance with our invention.

FIG. 3 is a photomicrograph of the graphite structure of a pipe cast after prolonged holding of a melt to which five nodularizing elements were added pursuant to our invention.

FIG. 4 is a graphical representation comparing the percentages of the original additions remaining in a bath of cast iron vs. holding time and comparing additions of one nodularizing element (as known in the prior art) to additions of more than one nodularizing element in accordance with our invention.

FIG. 5 is a graphical representation of the amount of two nodularizing elements remaining in pipe made under production condition vs. time after addition according to our invention.

**DETAILED DESCRIPTION OF THE INVENTION**

In FIG. 1 there is schematically represented the usual process for producing ductile iron castings. Our invention relates to the nodularizing step, those preceding steps being well known to one skilled in the art. The relationship between nodularizing agents used, the manner of use and the nodularizing effect forms the basis of our invention.

Our invention lies in the discovery that the total amount of nodularizing agents needed to produce ductile iron can be reduced if more than one nodularizing element is added in proper amounts. This allows a re-

duction in the concentration of the nodularizing elements in the bath which in turn improves efficiency, gives longer effective life, i.e., reduces fading, minimizes flare and smoke and minimizes the tendency for the iron to form dross.

The following results shown in Tables I and II were obtained from nodularizing individual heats of molten low sulfur cast iron as indicated:

TABLE I

| Test | Elements Added                | Total Amount Added                       | Total Remaining in Melt After:        |                                      |                                        |                                                            |
|------|-------------------------------|------------------------------------------|---------------------------------------|--------------------------------------|----------------------------------------|------------------------------------------------------------|
|      |                               |                                          | 1                                     | 5                                    | 10                                     | 15 - minutes                                               |
| A    | Mg                            | 0.05%                                    | .022                                  | .016                                 | .011                                   | .008                                                       |
| B    | Ce                            | 0.05%                                    | .037                                  | .019                                 | .011                                   | .003                                                       |
| C    | Mg+Ce                         | 0.05%                                    | .041                                  | .037                                 | .030                                   | .027                                                       |
|      | (0.025 Mg +<br>0.025 Ce)      |                                          | (.020)                                | (.017)                               | (.015)                                 | (.013) Mg - *                                              |
| D    | Mg<br>+Ce<br>+La<br>+Nd<br>+Y | 0.05%<br>(.01% of each<br>of 5 elements) | .034<br>.008<br>.008<br>.0085<br>.005 | .029<br>.007<br>.006<br>.006<br>.005 | .025<br>.006<br>.005<br>.0025<br>.0065 | .022<br>.005 Mg<br>.004 Ce<br>.001 La<br>.010 Nd<br>.002 Y |

\* - Numbers in Parentheses Represent Amount of Individual Elements

TABLE II

| Test | Element (s) Added   | Total Amount Added | % of Original Total Remaining in Melt |      |    |            |
|------|---------------------|--------------------|---------------------------------------|------|----|------------|
|      |                     |                    | 1                                     | 5    | 10 | 15 minutes |
| A    | Mg Only             | 0.05%              | 44                                    | 26.5 | 22 | 16         |
| B    | Ce Only             | 0.05%              | 74                                    | 38   | 22 | 6          |
| C    | Mg + Ce             | 0.05%              | 80                                    | 64   | 60 | 52         |
| D    | Mg+Ce+La<br>La+Nd+Y | 0.05%              | 69                                    | 58   | 50 | 44         |

In each test A through D as listed in the above Tables, the molten bath of low sulfur cast iron, prior to the nodularizing step, was comprised of the following elements within the ranges shown:

|              |                        |
|--------------|------------------------|
| Total Carbon | 3.4 - 3.6 per cent     |
| Silicon      | 1.9 - 2.1 per cent     |
| Manganese    | 0.25 - 0.30 per cent   |
| Sulfur       | 0.005 - 0.012 per cent |
| Phosphorus   | 0.04 - 0.06 per cent   |

In Test A the magnesium addition of 0.05 per cent by weight of iron was in the form of a commercial, cerium-free, magnesium ferrosilicon having a magnesium content of 6.17 per cent. In test B 0.05 per cent by weight of pure cerium metal chips was added to the bath. In test C the magnesium and cerium additions were made in the form of an alloy containing 3.0 per cent magnesium plus 3.0 per cent cerium, 45 per cent silicon, balance iron. The total nodularizing addition of 0.05 per cent by weight consisted of 0.025 per cent magnesium plus 0.025 per cent cerium. In test D, again the total nodularizing addition amounted to 0.05 per cent by weight. In this instance the nodularizing addition consisted of 0.01 per cent each of the following five elements: magnesium, cerium, lanthanum, neodymium and yttrium. Magnesium and cerium were added in the form of a ferrosilicon alloy containing 3 percent magnesium and 3 percent cerium. Lanthanum and neodymium were added in the metallic form; the neodymium contained 74 per cent neodymium and 14 per cent praseodymium. The yttrium was added in the form of a ferro silicon containing 20 per cent yttrium.

The results listed in Tables I and II are likewise shown graphically in FIGS. 1 and 2 where the amount of

nodularizer remaining in a bath of molten cast iron for each test A through D is plotted as a function of time, versus the amount of nodularizer originally added to the bath. It can be seen, from FIG. 2, that magnesium and cerium contents "fade" in time to lower and lower levels and at some point in time, the content is insufficient to produce a good spheroidal graphite structure. In the centrifugal casting of pipe in metal molds, we

have found that in cast irons having sulfur contents of the order of 0.004 to 0.006 per cent, the minimum range of magnesium content needed to insure a graphite structure in 6 inch diameter pipe in which approximately 90 per cent of the graphite consists of well-formed spheroids, is 0.012 to 0.014 per cent magnesium. In the case of cerium the required residual content has been found to be approximately 0.016 per cent. Thus, after 10 minutes holding time, neither magnesium nor cerium, when added alone as shown in curves A and B of FIG. 2, is present in sufficient quantities, in the melt, to insure the desired graphite structure, i.e. both quantities are below the "critical level."

In contrast to the behavior of magnesium or cerium when added individually in amounts of 0.05 per cent, the addition of smaller amounts (0.025 per cent) of magnesium and cerium together or 0.01 per cent of each of five nodularizing elements, results in more effective utilization of the nodularizing addition both from the standpoint of higher initial recoveries and longer effective life. Thus, it can be seen from curves C and D the total nodularizing content of the baths are over 0.02 per cent even at 15 minutes after addition.

We have further discovered that the various nodularizing elements differ in their nodularizing power when individually added to melts of cast iron; however, it appears that when added in combination, the combined total of the percentages of the nodularizing elements remaining in the melt can be used as an estimate of their nodularizing power in the melt.

As an illustration of this point, Table I shows the residual concentration of five nodularizing elements in a melt of cast iron at times up to 15 minutes after the addition of 0.01 percent of each element was made. A 6 inch diameter pipe was cast from this melt (Test D) at 18 minutes after the five elements were added. This pipe had an acceptable nodular graphite structure as shown in FIG. 3. Since the residual amounts of the individual nodularizing elements in this melt are so minute, as shown in Table I, the structure in FIG. 3 could only have resulted from the combined nodularizing power of all the elements present. It is also indicated in Table I that the sum total of nodularizing elements remaining

in the heat required to produce an acceptable graphite structure in pipe is of the same order of magnitude as (the residual amount of) magnesium alone or cerium alone (which would be required to produce the same acceptable graphite structure, as earlier stated).

The curves shown in FIG. 2 were established by adding only one of the nodularizing elements or combinations of the elements to baths of molten cast iron containing the following range of indicated elements in the final composition.

|              |                        |
|--------------|------------------------|
| Total Carbon | 3.4 - 3.6 per cent     |
| Silicon      | 2.7 - 2.9 per cent     |
| Manganese    | 0.25 - 0.30 per cent   |
| Sulfur       | 0.004 - 0.008 per cent |
| Phosphorus   | 0.04 - 0.06 per cent   |

The contents of Table II, which were derived from Table I, are shown graphically in FIG. 4 wherein the higher recovery of the nodularizers used pursuant to our invention over that of the prior art is again demonstrated.

In production tests magnesium plus cerium additions were made to 6-ton batches of iron in a ladle. The iron had the following analysis prior to the magnesium plus cerium additions.

|              |                        |
|--------------|------------------------|
| Total Carbon | 3.4 - 3.6 per cent     |
| Silicon      | 1.9 - 2.1 per cent     |
| Manganese    | 0.25 - 0.30 per cent   |
| Sulfur       | 0.005 - 0.012 per cent |
| Phosphorus   | 0.04 - 0.06 per cent   |

Data from these production tests are tabulated in Table III.

TABLE III

| Time From<br>Nodularizer<br>Addition Until<br>Pipe Was Cast | DATA FROM PRODUCTION TESTS |      |                               |                      |                   |             |                      |                    |
|-------------------------------------------------------------|----------------------------|------|-------------------------------|----------------------|-------------------|-------------|----------------------|--------------------|
|                                                             | %<br>Remaining<br>In Pipe  |      | Total<br>Remaining<br>In Pipe | Ultimate<br>Strength | Yield<br>Strength | %<br>Elong. | Charpy<br>Impact + % | Notched<br>- 40°F. |
|                                                             | Mg                         | Ce   | Mg + Ce                       |                      |                   |             |                      |                    |
| 9 1/2 mins.                                                 | .016                       | .007 | .023                          | 73,100               | 56,000            | 18.5        | 11.75                | 7.25               |
| 11 mins.                                                    | .014                       | .010 | .024                          | 75,300               | 58,800            | 17.5        | 10.75                | 5.25               |
| 12 1/2 mins.                                                | .016                       | .010 | .026                          | 75,400               | 58,400            | 15.5        | 9.25                 | 4.25               |
| 14 mins.                                                    | .016                       | .010 | .026                          | 73,800               | 56,900            | 17.0        | 8.50                 | 5.0                |
| 15 1/2 mins.                                                | .019                       | .006 | .025                          | 73,700               | 56,000            | 14.0        | —                    | —                  |
| 17 mins.                                                    | .015                       | .007 | .022                          | 71,500               | 53,900            | 17.0        | 10.75                | 6.5                |
| 6                                                           | .018                       | .015 | .033                          | —                    | —                 | —           | —                    | —                  |
| 24 1/2                                                      | .016                       | .007 | .023                          | 73,400               | 56,300            | 18.0        | 12.0                 | 6.5                |
| 26                                                          | .021                       | .008 | .029                          | 73,000               | 56,000            | 18.0        | 11.75                | 6.75               |
| 27 1/2                                                      | .015                       | .010 | .025                          | 73,000               | 56,000            | 18.0        | 12.25                | 6.0                |
| 29                                                          | .014                       | .013 | .027                          | —                    | —                 | —           | —                    | —                  |
| 31                                                          | .013                       | .011 | .024                          | 73,300               | 55,600            | 18.0        | 11.5                 | 6.5                |
| 32 1/2                                                      | .015                       | .012 | .027                          | —                    | —                 | —           | —                    | —                  |
| 34                                                          | .013                       | .010 | .024                          | 73,300               | 55,800            | 17.5        | 11.5                 | 5.5                |

The additions consisted of magnesium ferrosilicon (containing 5 per cent magnesium) plus an addition of cerium ferrosilicon (containing 10 per cent cerium). The amounts added were 0.025 per cent magnesium + 0.25 per cent cerium for a total nodularizing addition of 0.05 per cent. The tests showed that pipe having good spheroidal graphite structures could be cast at times as long as 34 minutes after the additions were made. The data illustrated in Table III is shown graphically in FIG. 5. The curves in FIG. 5 show that pipe cast 34 minutes after addition of magnesium + cerium were

found to contain 0.013 per cent magnesium + 0.010 per cent cerium. The salient feature of these data is that neither element is present in sufficient quantity to insure the production of good spheroidal graphite structures by itself; however, the combined total content of nodularizing elements (0.023 per cent) is sufficient to produce the desired graphite structure. This is also illustrative of the efficiency and longer effective life obtained by small additions of nodularizing elements since the residual content of magnesium + cerium (0.023 per cent) represents a recovery of 46 per cent of the original total nodularizing addition 34 minutes after the addition was made. Also included in Table III are the results of mechanical tests which are indicative of the structures obtained in the pipe. These pipe met the stringent requirements of commercial specifications for notched impact resistance as well as tensile properties.

Another series of tests were conducted under production conditions to determine whether or not the results obtained by the combined addition of two separate alloys (magnesium ferrosilicon plus cerium ferrosilicon) could be obtained by the addition of one alloy containing both magnesium and cerium. In these tests 6-ton batches of cast iron were treated with additions of an alloy containing 2.5 per cent magnesium plus 2.4 per cent cerium. In one test an addition of 0.83 per cent of this alloy, by weight, was made. This amounted to an addition of 0.021 per cent magnesium plus 0.020 per cent cerium, for a total nodularizing addition of 0.041 per cent. In this test 8 inch diameter pipe, cast 31 minutes after a nodularizing treatment, contained 0.011 per cent magnesium plus 0.012 per cent cerium for a total of 0.023 per cent (magnesium + cerium). This represents a recovery 56 per cent of the original amount, and verifies that the high recoveries and

longer effective life of the nodularizing elements can be obtained by the simultaneous addition of separate alloys each containing a nodularizer, or by the addition of one alloy containing more than one nodularizer. In these plant trials using the alloy containing 2.5 per cent magnesium + 2.4 per cent cerium, the flaring and evolution of smoke generally associated with adding magnesium-containing alloys were virtually eliminated.

From the foregoing it is apparent that the addition of an alloy or mixture of alloys containing not more than 3% of each of two or more nodularizers in small quanti-

ties will assure that sufficient nodularizers will be present over a longer period of time than when the same total quantity of one nodularizer is added and will eliminate any violent reaction accompanying the addition. This phenomenon is quite surprising and is not fully understood.

In experiments using this 2.5 percent magnesium + 2.4 percent cerium alloy for making sand castings it was found that acceptable graphite structures could be produced with additions of nodularizing elements that were 20 percent less than required with a conventional 5 percent magnesium ferrosilicon. With this reduction less alloy addition is required and this in turn reduces the amount of dross formed.

Although the preferred embodiment of the present invention has been described, it will be understood that it is intended to cover all changes and modifications of the invention herein chosen for the purpose of illustration which do not constitute departures from the spirit and scope of the invention.

We claim:

1. A nodularizing composition for use in the production of nodular cast iron comprising at least two nodularizing elements in a silicon-iron alloy or mixture of silicon-iron alloys, said elements selected from the group consisting of magnesium, cerium, yttrium, lanthanum, neodymium and praseodymium with each being present in the alloy or alloys in an amount of from about 1 to 3 percent by weight of the composition and the total amount of nodularizing elements in the

30

composition not exceeding more than about 12 percent.

2. The composition of claim 1 wherein the nodularizing elements are magnesium and cerium in substantially equal amounts.

3. A nodularizing composition for use in the production of nodular cast iron comprising at least two silicon-iron alloys, one alloy containing magnesium in an amount of from about 1 to 3 percent by weight and the other alloy comprising at least one nodularizing element selected from the group consisting of cerium, yttrium, lanthanum, neodymium and praseodymium with each being present in an amount of from about 1 to 3 percent by weight of the alloy and the total amount of nodularizing elements in the composition not exceeding more than about 12 percent.

4. A nodularizing composition for use in the production of nodular cast iron comprising at least two nodularizing elements and one of said at least two nodularizing elements being magnesium and being present in a silicon-iron alloy from about 1 to 3 percent by weight of the composition and the remainder of said at least two nodularizing elements selected from the group consisting of cerium, yttrium, lanthanum, neodymium and praseodymium, each being present in about the same amount as said magnesium and the total amount of nodularizing elements in the composition not exceeding more than about 12 percent.

\* \* \* \* \*

35

40

45

50

55

60

65

UNITED STATES PATENT OFFICE  
CERTIFICATE OF CORRECTION

PATENT NO. : 3,905,809

DATED : September 16, 1975

INVENTOR(S) : Andrew B. Malizio, Martin A. Rice & Harry F. Brooks

It is certified that error appears in the above-identified patent and that said Letters Patent are hereby corrected as shown below:

Col. 3, Table II, Test D should read:

-- Mg + Ce + La + Nd + Y --.

Signed and Sealed this  
twenty-third Day of December 1975

[SEAL]

Attest:

RUTH C. MASON  
Attesting Officer

C. MARSHALL DANN  
Commissioner of Patents and Trademarks

**REEXAMINATION CERTIFICATE (746th)**  
**United States Patent [19]**  
**Malizio et al.**

[11] B1 3,905,809

[45] Certificate Issued Aug. 18, 1987

**[54] ALLOY FOR MAKING DUCTILE IRON**

- [75] Inventors: **Andrew B. Malizio, Delran; Martin A. Rice, Florence, both of N.J.; Harry F. Brooks, Levittown, Pa.**  
[73] Assignee: **United States Pipe and Foundry Company, Birmingham, Ala.**

**Reexamination Request:**

No. 90/001,157, Jan. 30, 1987

**Reexamination Certificate for:**

Patent No.: **3,905,809**  
Issued: **Sep. 16, 1975**  
Appl. No.: **434,403**  
Filed: **Jan. 18, 1974**

Certificate of Correction issued Dec. 23, 1975.

**Related U.S. Application Data**

- [62] Division of Ser. No. 189,670, Oct. 15, 1971, Pat. No. 3,799,767.  
[51] Int. Cl.<sup>4</sup> ..... C22C 37/00  
[52] U.S. Cl. ..... 420/578; 75/53;  
420/25  
[58] Field of Search ..... 75/53; 420/25, 578

[56] **References Cited**

**U.S. PATENT DOCUMENTS**

- 1,555,978 10/1925 Hunt ..... 75/130 A  
2,542,655 2/1951 Gagnebin et al. ..... 75/130 A X  
2,555,014 5/1951 Strauss ..... 75/138 A X

|           |         |                         |            |
|-----------|---------|-------------------------|------------|
| 2,792,300 | 5/1957  | Livingston .....        | 75/130 A   |
| 2,814,559 | 11/1957 | Clark .....             | 75/53      |
| 2,816,829 | 12/1957 | Bogart .....            | 75/130     |
| 2,816,829 | 12/1957 | Bogart .....            | 75/130     |
| 2,841,488 | 7/1958  | Morrogh .....           | 75/123     |
| 2,841,489 | 7/1958  | Morrogh .....           | 75/125 A X |
| 2,841,490 | 7/1958  | Steven et al. ....      | 75/130 C   |
| 2,867,555 | 1/1959  | Curry .....             | 75/130 A X |
| 2,873,188 | 2/1959  | Bieniosek .....         | 75/130 A   |
| 2,877,111 | 3/1959  | Barnes, Jr. et al. .... | 75/130 C   |
| 3,155,498 | 11/1964 | Jandras .....           | 75/130 C   |
| 3,336,118 | 8/1967  | Newitt .....            | 29/192     |
| 3,459,541 | 8/1969  | Hohl et al. ....        | 75/130 A   |
| 3,492,118 | 1/1970  | Mickelson .....         | 75/130     |

**FOREIGN PATENT DOCUMENTS**

827166 2/1960 United Kingdom

**OTHER PUBLICATIONS**

Modern Castings, Oct. 1965, pp. 442-445, "Influence of Magnesium Content on the Nodularizing Efficiency of Magnesium Ferrosilicon Alloys".

*Primary Examiner*—Peter D. Rosenberg

[57] **ABSTRACT**

A process for producing ductile iron comprising adding to a bath of low-sulfur cast iron, a material containing at least two graphite-nodularizing elements. The additive material contains each nodularizing element in relatively low concentrations so that after dissolution in the bath the concentration of nodularizing elements remaining is sufficient to produce the desired structure, but the concentration of any one element is, of itself, insufficient to produce nodular (spheroidal) graphite.

**REEXAMINATION CERTIFICATE  
ISSUED UNDER 35 U.S.C. 307**

THE PATENT IS HEREBY AMENDED AS  
INDICATED BELOW.

Matter enclosed in heavy brackets **[ ]** appeared in the patent, but has been deleted and is no longer a part of the patent; matter printed in italics indicates additions made to the patent.

AS A RESULT OF REEXAMINATION, IT HAS  
BEEN DETERMINED THAT:

Claims 1, 3 and 4 are determined to be patentable as amended.

Claim 2, dependent on an amended claim, is determined to be patentable.

New claims 5-8 are added and determined to be patentable.

1. A nodularizing composition for use in the production of nodular cast iron **[comprising]** consisting essentially of at least two nodularizing elements in a silicon-iron alloy or mixture of silicon-iron alloys, said elements selected from the group consisting of magnesium, cerium, yttrium, lanthanum, neodymium and praseodymium with each being present in the alloy or alloys in an amount of from about 1 to 3 percent by weight of the composition and the total amount of nodularizing elements in the composition not exceeding more than about 12 percent.

3. A nodularizing composition for use in the production of nodular cast iron **[comprising]** consisting essentially of at least two silicon alloys, one alloy **[containing]** consisting essentially of magnesium in an amount of from about 1 to 3 percent by weight and the other alloy **[comprising]** consisting essentially of at least one nodularizing element selected from the group consisting of cerium, yttrium, lanthanum, neodymium and praseodymium with each being present in an amount of from about 1 to 3 percent by weight of the alloy and the total

35  
40  
45

amount of nodularizing elements in the composition not exceeding more than about 12 percent.

4. A nodularizing composition for use in the production of nodular cast iron **[comprising]** consisting essentially of at least two nodularizing elements and one of said at least two nodularizing elements being magnesium and being present in a silicon-iron alloy from about 1 to 3 percent by weight of the composition and the remainder of said at least two nodularizing elements selected from the group consisting of cerium, yttrium, lanthanum, neodymium and praseodymium, each being present in about the same amount as said magnesium and the total amount of nodularizing elements in the composition not exceeding more than about 12 percent.

5. *A nodularizing composition for use in the production of nodular cast iron comprising at least two nodularizing elements in a silicon-iron alloy or mixture of silicon-iron alloys, said elements selected from the group consisting of magnesium, cerium, yttrium, lanthanum, neodymium and praseodymium with each being present in the alloy or alloys in an amount of from about 1 to 2.9 percent by weight of the composition and the total amount of nodularizing elements in the composition not exceeding more than about 12 percent.*

6. *The composition of claim 5 in which the nodularizing elements are magnesium and cerium in substantially equal amounts.*

7. *A nodularizing composition for use in the production of nodular cast iron comprising at least two silicon-iron alloys, one alloy containing magnesium in an amount of from about 1 to 2.9 percent by weight and the other alloy comprising at least one nodularizing element selected from the group consisting of cerium, yttrium, lanthanum, neodymium and praseodymium with each being present in an amount of from about 1 to 2.9 percent by weight of the alloy and the total amount of nodularizing elements in the composition not exceeding more than about 12 percent.*

8. *A nodularizing composition for use in the production of nodular cast iron comprising at least two nodularizing elements and one of said at least two nodularizing elements being magnesium and being present in a silicon-iron alloy from about 1 to 2.9 percent by weight of the composition and the remainder of said at least two nodularizing elements selected from the group consisting of cerium, yttrium, lanthanum, neodymium and praseodymium, each being present in about the same amount as said magnesium and the total amount of nodularizing elements in the composition not exceeding more than about 12 percent.*

\* \* \* \* \*

50

55

60

65

**REEXAMINATION CERTIFICATE (1287th)**  
**United States Patent [19]** [11] **B2 3,905,809**  
**Malizio et al.** [45] **Certificate Issued May 29, 1990**

---

[54] **ALLOY FOR MAKING DUCTILE IRON**

[56] **References Cited**

**U.S. PATENT DOCUMENTS**

2,542,655 2/1951 Gagnebin et al.  
2,841,488 7/1958 Morrogh

**FOREIGN PATENT DOCUMENTS**

1126013 9/1968 United Kingdom

**OTHER PUBLICATIONS**

"Influence of Magnesium Content on the Nodularizing Efficiency of Magnesium-Ferrosilicon Alloys", Clark et al., *Modern Castings*, Oct. 1965, pp. 442-445.

"The Use of Multiple Nodularizing Elements in Making Ductile Iron Pipe", Rice et al., *AFS Transactions*, pp. 15-26 (1974).

*Primary Examiner*—Peter D. Rosenberg

[57] **ABSTRACT**

A process for producing ductile iron comprising adding to a bath of low-sulfur cast iron, a material containing at least two graphite-nodularizing elements. The additive material contains each nodularizing element in relatively low concentrations so that after dissolution in the bath the concentration of nodularizing elements remaining is sufficient to produce the desired structure, but the concentration of any one element is, of itself, insufficient to produce nodular (spheroidal) graphite.

[73] **Assignee:** **United States Pipe and Foundry Company, Birmingham, Ala.**

**Reexamination Request:**  
No. 90/001,270, Jun. 29, 1987

**Reexamination Certificate for:**

Patent No.: 3,905,809  
Issued: Sep. 16, 1975  
Appl. No.: 434,403  
Filed: Jan. 18, 1974

Reexamination Certificate B1 3,905,809 issued Aug. 18, 1987.

[51] **Int. Cl.<sup>5</sup>** ..... C22C 37/00  
[52] **U.S. Cl.** ..... 420/578; 75/53;

420/25

[58] **Field of Search** ..... 420/578, 25; 75/53

**REEXAMINATION CERTIFICATE  
ISSUED UNDER 35 U.S.C. 307**

THE PATENT IS HEREBY AMENDED AS  
INDICATED BELOW.

AS A RESULT OF REEXAMINATION, IT HAS  
BEEN DETERMINED THAT:

5      Claims 1-8 are cancelled.

\* \* \* \* \*

10

15

20

25

30

35

40

45

50

55

60

65